

Oct. 16, 1923.

1,471,190

H. A. MYERS

PROCESS OF PRODUCING SOFT FERROUS METAL CASTINGS

Filed Sept. 23, 1921



FIG. 1.



FIG. 2.

INVENTOR

*Hubert A. Myers.*  
by  
*Owen, Owen & Campbell.*

Patented Oct. 16, 1923.

1,471,190

# UNITED STATES PATENT OFFICE.

HUBERT A. MYERS, OF TOLEDO, OHIO, ASSIGNOR TO THE HUBERT A. MYERS COMPANY, OF TOLEDO, OHIO, A CORPORATION OF OHIO.

## PROCESS OF PRODUCING SOFT FERROUS METAL CASTINGS.

Application filed September 23, 1921. Serial No. 502,637.

To all whom it may concern:

Be it known that I, HUBERT A. MYERS, a citizen of the United States, and a resident of Toledo, Lucas County, Ohio, have made an Invention Appertaining to Process of Producing Soft Ferrous Metal Castings; and I do hereby declare the following to be a full, clear, and exact description of the invention, such as will enable others skilled in the art to which it appertains to make and use the same, reference being made to the drawings, and to the characters of reference marked thereon, which form a part of this specification.

15 My invention relates to the process of producing soft ferrous castings. It particularly has for its object to prevent crystallization, thus avoiding the production of stresses and strains within the castings; 20 avoiding the formation of hardening carbon and of carbide carbon and allowing substantially a complete liberation of the carbon from its solution with the metal as the metal cools, thus permitting substantially 25 all of the carbon to become free carbon before the metal solidifies.

The invention may be carried out in apparatus of different forms. To illustrate a practical application of the invention I have shown in the accompanying drawings an apparatus in which the process may be conducted and I shall describe the apparatus in connection with the process.

Figure 1 illustrates a top view of the apparatus, and Fig. 2 illustrates a side view.

35 1 is a molding machine that may be hand operated by the crank 2 to open and close the parts 3 and 4 of the mold that correspond to the drag and the cope of a mold. 40 A pair of arms 5 may be connected to the crank 2 and a pair of ears 6 may be connected to the part 3 of the mold and links 7 may be used to connect the arms 5 with the ears 6, so that when the crank 2 is oscillated 45 the part 3 will be moved along the guides 18 to open or close the mold. The mold 8 may, if desired, be heated by a flame from the nozzle 9 or the temperature of the mold may be raised and controlled by the rate at which 50 the pourings are made. The temperature of the mold to obtain the best results is preferably kept at such a point that the metal will not fall below 1300° F. The walls that form the matrix of the mold may be made of any

material that will withstand the temperature and permit the rapid formation of the castings within the mold. The temperature of the mold may be regulated by any other method or means.

55 The castings may be ejected from the mold, when the parts 3 and 4 have been separated, by any suitable means and allowed to fall upon the inclined trough 10, which will direct them to the inlet or opening of the lehr. They may be directed onto a conveyer 12 formed of a suitable material to withstand the high temperature at which the lehr is maintained and to which the castings are subjected while within the lehr. Any form 60 of means may be provided for conveying or directing the castings from the mold into the lehr. It is, however, desirable that the transfer be made with quickness in order to prevent chilling of the castings. In order 65 to avoid the cooling effect in the transfer of the castings from the mold to the lehr the mold may be placed at the mouth of the lehr.

70 The conveyer 12 may be of any form and the one shown in the drawings is merely a conventional illustration of a means for permitting successive castings to be carried into the lehr and maintained in the lehr for a considerable length of time so that the temperature of the castings as they 75 pass through the lehr may be so controlled that the carbon will have an opportunity to become liberated from the solution that it forms with the iron. The lehr is heated by a plurality of burners 13 and the temperature 80 produced by the burners is controlled by any means, such as by the valves 14, so as to permit a very gradual reduction of the temperature while the castings are carried slowly 85 through the lehr by means of the conveyer 12 and finally removed from the conveyer 12 when the temperature is well below 1300° F., such as below 900° F.

90 The castings may be discharged from the lehr at a temperature somewhat above 900° F. if provision is made for slow subsequent 95 cooling of the castings. They may be discharged into a comminuted heat insulating material such as flaked mica contained in a trough or receptacle of any suitable form. 100 In the apparatus illustrated I have shown 105 a conveyer containing a plurality of containers or boxes 15 linked together and sup-

ported on tracks 16 by means of rollers or wheels 17 and containing flaked mica or other heat insulating powdered material in which the castings will be practically submerged by the impact caused by dropping them from the conveyer 12. The castings may thus be conveyed from the lehr and the slow cooling of the castings continued after leaving the lehr.

10 The soft castings will thus be formed without permitting crystallization or formation of cementite at any time since the slow cooling from the time the metal is first poured prevents the combination of 15 the carbon with the iron. In this way better castings are formed than when castings are annealed as in the process commonly used in making malleable castings.

I claim:—

20 1. The process of producing soft ferrous castings, which consists in shaping the castings in a hot mold, delivering the castings from the mold before the temperature of the castings decreases sufficiently to prevent dissolution of the carbon in the metal, and maintaining the lehr and the castings at a temperature higher than that at which carbon will combine with the iron until substantially all of the carbon has become liberated from the solution and allowing the castings to gradually cool.

25 2. The process of producing soft ferrous castings, which consists in shaping the castings in a hot mold directing the castings from the mold to a lehr before the temperature of the castings decreases sufficiently to prevent dissolution of the carbon in the metal, a portion of the lehr being maintained at a temperature higher than 30 that at which carbon will combine with the iron, and retaining the castings in the lehr until substantially all of the carbon has

become liberated from its solution with the metal.

3. The process of producing soft ferrous 45 castings, which consists in shaping the castings in a hot mold, directing the castings from the mold to a lehr before the temperature of the castings decreases sufficiently to prevent dissolution of the carbon in the metal, a portion of the lehr being maintained at a temperature higher than that at which carbon will combine with the iron until substantially all of the carbon has been liberated from solution with the 50 ferrous metal and substantially submerging the castings in powdered heat insulating material upon their discharge from the lehr.

4. The process of producing soft ferrous 55 castings, which consists in shaping the castings in hot molds, directing the castings from the molds to a lehr before the temperature of the castings decreases sufficiently to prevent dissolution of the carbon in the metal, the lehr being maintained 60 at a temperature higher than that at which carbon will combine with the iron and retaining the castings in the lehr until substantially all of the carbon has become liberated from its solution with the metal, substantially submerging the castings in flaked 65 mica upon their discharge from the lehr.

5. In an apparatus for producing soft ferrous metal castings, a casting means, a lehr, a conveyer, movable within the lehr, 75 means for conveying the castings from the casting means to the conveyer, means for heating and regulating the temperature of the lehr, a receptacle for receiving the castings from the lehr, and a heat insulating 80 material located within the receptacle.

In testimony whereof I have subscribed my name to this specification.

HUBERT A. MYERS.